

# United States Patent

[19]

Curtin

[11] 3,928,035

[45] Dec. 23, 1975

[54] ELECTROPHOTOGRAPHIC ELEMENT  
WHICH INCLUDES A PHOTOCONDUCTIVE  
POLYVINYL CARBAZOLE LAYER  
CONTAINING AN AROMATIC ANHYDRIDE

[75] Inventor: Denis J. Curtin, Chicago, Ill.

[73] Assignee: A. B. Dick Company, Niles, Ill.

[22] Filed: June 7, 1974

[21] Appl. No.: 477,301

[52] U.S. Cl..... 96/1.5; 252/501

[51] Int. Cl.<sup>2</sup>..... G03G 5/04

[58] Field of Search..... 96/1.5 C; 252/501

[56] **References Cited**

UNITED STATES PATENTS

|           |         |                     |         |
|-----------|---------|---------------------|---------|
| 3,484,237 | 12/1969 | Shattuck et al..... | 252/501 |
| 3,764,311 | 10/1973 | Bean .....          | 96/1.5  |
| 3,798,030 | 3/1974  | Gundlach.....       | 96/1.5  |

## OTHER PUBLICATIONS

Nepela et al., IBM Technical Disclosure Bulletin, Sensitization of Organic Photoconductor Complexes Using Quinones, Vol. 13, No. 5, Oct. 1970.

*Primary Examiner*—Mary F. Kelley

*Assistant Examiner*—Judson R. Hightower

[57] **ABSTRACT**

For use in an electrophotographic copy process, a photoconductive element comprising a support for an organic photoconductive coating comprising a polymerized vinyl carbazole, 2,4,7-trinitro-9-fluorenone and an aromatic anhydride present in amounts of about 0.49 to 1.23 moles of the trinitrofluorenone per monomeric unit of polyvinyl carbazole and 0.05 to 5.0 percent by weight of aromatic anhydride based upon the amount of polyvinyl carbazole.

**12 Claims, No Drawings**

**ELECTROPHOTOGRAPHIC ELEMENT WHICH INCLUDES A PHOTOCONDUCTIVE POLYVINYL CARBAZOLE LAYER CONTAINING AN AROMATIC ANHYDRIDE**

This invention relates to photoconductors and more particularly to an organic photoconductor composition for use in the preparation of photoconductive elements in the production of copy by the electrophotographic process.

In the electrophotographic copy process, use is made of a photoconductive surface onto which a uniform electrostatic charge is applied. The charge is retained on the surface except for those areas that are rendered conductive during exposure to a light pattern, leaving a latent electrostatic image on the non-exposed portions of the photoconductive surface. The latent electrostatic image is subsequently developed in a conventional manner, as by means of a dry developing powder which is cascaded over the surface, or by a liquid developer or toner suspended in an insulating liquid with which the plate surface is wet. Instead, the latent electrostatic image can be transferred to a copy sheet for development of the image thereon, as by a liquid or powder developer.

To the present, especially in relatively high speed copy machines, amorphous selenium, with or without an added dopant, has been used to provide the photoconductive surface on a suitable support. While selenium provides a photoconductive surface having the desired speed and sensitivity for use in high speed copy machines, selenium represents a relatively expensive material which is difficult to apply, and its use as a photoconductive composition is somewhat restricted to a support formed of a rigid material such as a metal drum or plate.

There is considerable interest in a low cost organic photoconductive composition which might be applied by conventional coating techniques, for use on various supports, such as on an endless belt, flexible paper, metal or plastic strip, and the like, as well as on a rigid metal drum or plate.

While organic photoconductors offer advantages of the type described, they are also faced with a number of disadvantages in that organic photoconductors, which have been suggested to the present, are characterized by low charge acceptance and lesser sensitivity by comparison with selenium.

In U.S. Pat. No. 3,484,237, description is made of an organic photoconductor composition formed of a polymerized vinyl carbazole compound to which 2,4,7-trinitro-9-fluorenone has been added as an electron acceptor to lower the dark conductivity of the photoconductive layer and to increase the sensitivity in the visible range.

It is an object of this invention to increase the photoconductivity, charge acceptance, and sensitivity of photoconductive compositions of the type described in the aforementioned U.S. Pat. No. 3,484,237, whereby the photoconductive element embodying the advantages available from the use of an organic photoconductor composition and the speed and sensitivity comparable to a photoconductor formed of selenium is obtained.

More specifically, it is an object of this invention to provide an organic photoconductor composition from which a photoconductor can be produced having good

charge acceptance, good photoconductive speed for use in the production of copies at high speed on conventional copy machines, which can be applied for use in providing a photoconductive coating on a rigid or on a flexible support, and which can be formulated of relatively low cost and readily available material for application by conventional coating means to produce a low cost electrophotographic element.

It has been found, in accordance with the practice of this invention, that the photoconductivity, charge acceptance and sensitivity or the speed of a photoconductive composition formulated of 2,4,7-trinitro-9-fluorenone (TNF) and a polymerized vinyl carbazole (PVK) present in the ratio of about 0.49 to 1.3 moles of TNF per monomer unit of PVK can be improved when addition is made of an aromatic anhydride. By the addition of aromatic anhydride, the charge acceptance of the photoconductive layer can be increased by at least 25% and the sensitivity of the photoconductive coating can be increased three to eight fold or more with corresponding increase in copy speed by comparison with the same composition without the added aromatic anhydride. This represents a significant improvement whereby copy speed and quality suitable for high speed copy machines can be achieved.

Polymerized vinyl carbazole compounds suitable for use in the photoconductive compositions of this invention are poly-N-vinyl carbazole and polyvinyl-N-lower alkyl carbazoles of the type described in the U.S. Pat. No. 3,484,237. The following can be given by way of examples of suitable poly-N-lower alkyl carbazoles, namely, poly-2-vinyl-N-methylcarbazole, poly-3-vinyl-N-ethylcarbazole, poly-2-vinyl-N-ethylcarbazole, poly-3-vinyl-N-methylcarbazole, poly-3-vinyl-N-isopropylcarbazole, poly-2-vinyl-N-butylcarbazole, poly-3-vinyl-N-butylcarbazole, poly-2-vinyl-N-pentylcarbazole, poly-3-vinyl-N-pentylcarbazole, poly-2-vinyl-N-hexylcarbazole, poly-3-vinyl-N-hexylcarbazole, poly-2-vinyl-N-heptylcarbazole, and poly-3-vinyl-N-heptylcarbazole. Mixtures and copolymers of the polymerized vinyl-carbazole compounds also may be used.

Representative of the aromatic anhydrides which can be used in the practice of the invention are phthalic anhydride (PA), 1,2,4,5-benzene-tetracarboxylic anhydride (BT), mellitic trianhydride (MT), and the like anhydrides of dicarboxylic, tricarboxylic, tetracarboxylic and polycarboxylic benzyl, naphthyl, and anthracetyl, or other unsubstituted or substituted aromatic ring structures. The desired improvements are experienced when the phthalic anhydride, mellitic trianhydride, 1,2,4,5-benzene-tetracarboxylic anhydride, or other aromatic anhydrides is present in the photoconductive composition in an amount within the range of 0.05 to 5.0, and preferably 0.90 to 1.7 percent by weight of the polyvinylcarbazole component.

The materials are formulated into a composition for coating onto a suitable substrate by first dissolving the polyvinylcarbazole component in a suitable solvent, such as tetrahydrofuran, and then admixing the solution of the polyvinylcarbazole with the 2,4,7-trinitro-9-fluorenone and aromatic anhydride, preferably in solution in the same solvent, and any additional solvent required to achieve the desired consistency for the coating composition. The materials may be worked into solution on a roller mill and the like and coated on a suitable substrate, such as a paper plate, silicated aluminum plate, or the like, by conventional coating means, followed by air drying and then curing at ele-

vated temperature such as for one hour at 50°-60°C.

Instead of tetrahydrofuran, other solvents such as 1,2-dichloroethane and chlorobenzene may be used.

The photoconductive compositions of the present invention are useful in the conventional xerographic process in which an electrostatic image is formed on the surface of the photoconductive element and the electrostatic image is subsequently developed. In practice, the photoconductive element is electrostatically charged and exposed to a pattern of light and dark to form an electrostatic image. Thereafter, the electrostatic image can either be developed with a conventional electroscopic powder developer on the photoconductive element and the developed image transferred to plain paper, or the electrostatic image can be transferred to a dielectric paper for development with an electroscopic developer (powder or liquid). The following examples will illustrate the improvement that is achieved by the addition of the aromatic anhydride to the organic photoconductor composition in accordance with the practice of this invention.

#### EXAMPLES 1 to 4

In the following examples, a photoconductive coating formulated of 2,4,7-trinitro-9-fluorenone (TNF) and poly-N-vinylcarbazole (PVK) in the amount described will be compared with coatings of the same composition but with the addition of the same amounts of various aromatic anhydrides, representative of the practice of this invention. Comparisons will be made from the standpoint of initial charge, and residual charge in volts, dark decay in volts per second, and sensitivity at light exposures of 7, 14 and 28  $\mu$  J/cm<sup>2</sup>.

For this purpose, a master mix was prepared of 24.8 grams 2,4,7-trinitro-9-fluorenone from Aldrich Chemical Co. Inc., 575 ml tetrahydrofuran previously dried over sodium, 160 ml of 10% solution in tetrahydrofuran of poly-N-vinyl-carbazole from Ionac Chemical Company.

The solution of the above materials was divided into four equal segments, identified as Examples 1, 2, 3, and 4. In Example 1, no addition was made. In Example 2, 0.5 ml of 1% by weight solvent solution in tetrahydrofuran of phthalic anhydride was added. In Example 3, 0.5 ml of a 1% solution in tetrahydrofuran of 1,2,4,5-benzene-tetracarboxylic anhydride was added. In Example 4, addition was made of 0.5 ml of a 1% solution in tetrahydrofuran of mellitic anhydride.

The compositions of each of the four examples were milled on a roller immediately prior to coating. The compositions of Examples 1-4 were each applied onto 3.5 mil silicated aluminum substrate with a Paasche H-5 artist air brush. For this purpose, the aluminum plate was mounted onto a drum supported for rotational movement about a horizontal axis. The air brush was attached to a rack and pinion mechanism which allowed the air brush to be moved across the width of the plate at a fixed plate surface to air brush distance.

During rotation of the drum at about 13 rpm, a narrow strip of coating was applied by the air brush, using nitrogen gas. After each rotation, the air brush was moved about 2 mm and another strip was applied until the aluminum plate was covered with a thin coating to a coating thickness of 5-20 microns, and preferably 8-15 microns. The plates were allowed to air dry and then the coating was cured for 60 minutes at 50°C.

The plates were subjected to tests for acceptance and retention of electrostatic charge, including charge

decay in the dark. For this purpose, the plates were each exposed to a negative electrostatic corona charge of 6 KV by passing the plate beneath charging wires and the charged plates were tested for initial voltage, residual charge, dark decay and sensitivity. Initial charge, charge retention and charge acceptance were measured by a Monroe electrometer which measures the charge on the surface of the plate. Dark decay was calculated by the rate of charge loss per second. Sensitivity was determined by the Monroe electrometer to calculate the amount of charge dissipated by light upon exposure. Exposure was made with a tungsten photo enlarger lamp (150 W) operating through an enlarger. Energy of exposure identifies the amount of light that fell on the plate  $\mu$  J/cm<sup>2</sup> as measured by a Hewlett-Packard radiant flux meter.

TABLE I

| Example | Additive                                  | Initial charge (V) | Residual charge (V) | Dark decay (V/sec) |
|---------|-------------------------------------------|--------------------|---------------------|--------------------|
| 1       | None                                      | 140                | 24                  | 2.2                |
| 2       | Phthalic anhydride                        | 300                | 30                  | 3.3                |
| 3       | 1,2,4,5-benzene-tetracarboxylic anhydride | 500                | 30                  | 1.5                |
| 4       | Mellitic anhydride                        | 600                | 30                  | 3.3                |

It will be seen from the above results that the additions of aromatic anhydride operated effectively to increase the initial charge and the residual charge retained on the photoconductor.

The plates were also tested for sensitivity by uniform exposure to the tungsten lamp for various exposures ranging from 7, 14 and 28  $\mu$  J/cm<sup>2</sup>, with the following results expressed in V cm<sup>2</sup>/ $\mu$  J:

TABLE II

| Example | 7    | Exposure 14 | 28   | Average sensitivity | Percent Improvement |
|---------|------|-------------|------|---------------------|---------------------|
|         |      | sensitivity |      |                     |                     |
| 1       | 4.0  | 3.3         | 2.5  | 3.3                 | —                   |
| 2       | 12.9 | 10.0        | 7.1  | 10.0                | 303                 |
| 3       | 22.9 | 15.6        | 12.9 | 18.1                | 548                 |
| 4       | 28.6 | 23.2        | 16.1 | 26.6                | 806                 |

From the results on sensitivity, it will be seen that the additions of aromatic anhydrides resulted in a three to eight fold increase in the sensitivity of the photoconductor, permitting a three to eight fold increase in speed. This corresponds to a reduction in copy time for the photoconductor with the added aromatic anhydride when compared to a photoconductor of the same composition without added aromatic anhydride. This marked increase in light sensitivity of the photoconductor composition permits the elimination of activator, such as the undesirable dyestuffs heretofore employed in compositions of the type described, without loss of copy speed or copy quality.

The following are further examples of the practice of this invention with various aromatic anhydrides added to the system of 2,4,7-trinitro-9-fluorenone and poly-N-vinyl-carbazole in varying amount.

#### EXAMPLE 5

6.2 grams TNF  
40.0 ml of 10% poly-N-vinylcarbazole in tetrahydrofuran (THF)  
60.0 ml THF

5.0 ml of a 1% solution of phthalic anhydride in THF

EXAMPLE 6

10 grams TNF

100 ml THF

65 ml of 10% solution of poly-N-vinylcarbazole in THF

4.8 ml of a 1% solution of phthalic anhydride in THF

EXAMPLE 7

6.2 grams TNF

40.0 ml of 10% solution of poly-N-vinylcarbazole in THF

60.0 ml THF

0.5 ml of a 1% solution of BT in THF

EXAMPLE 8

6.2 grams of TNF

60.0 ml THF

40.0 ml 10% solution of poly-N-vinylcarbazole in THF

0.5 ml of a 1% solution of MT in THF

The formulations of Examples 5 to 8 were roller milled until the material became dissolved in the THF. 25 The milled compositions were each coated on a substrate in the form of a silicated aluminum plate having a thickness of 0.0035 inch. The photoconductive coating compositions of Examples 5 to 8 were applied by the meniscus coating method in coating thickness of 30 5-20 microns, and preferably 8-15 microns. The coated plates were allowed to air dry and then cured for one hour at 60°C.

The following is a tabulation comparing the electrical properties of the plates prepared in Examples 5 to 8, compared with a plate prepared in the same way, with a similar photoconductor composition, but without the added aromatic anhydride:

TABLE III

|                         | Charge Acceptance (volts) | Energy of Exposure $\mu\text{J/cm}^2$ | Sensitivity $\text{Vcm}^2/\mu\text{J}$ |
|-------------------------|---------------------------|---------------------------------------|----------------------------------------|
| PVK-TNF (w/O anhydride) | 450                       | 7.0                                   | 17.5                                   |
| Example 5               | 750                       | 7.5                                   | 33.5                                   |
| Example 6               | 800                       | 7.0                                   | 42.8                                   |
| Example 7               | 1100                      | 7.0                                   | 60                                     |
| Example 8               | 1000                      | 7.0                                   | 57                                     |

The plates of Example 6 were imaged by cascading a commercial IBM powder developer over the surface of the imaged plate. The toned image was transferred to bond paper by the use of a negative corona, in accordance with conventional practice, and then exposed to an IR lamp for a time sufficient to heat the toner particles to fusion to set the image. Copy of good quality was secured in times corresponding to that experienced in commercial practice with selenium plates. 50

It will be understood that changes may be made in the details of formulation and operation, without de-

parting from the spirit of the invention, especially as defined by the following claims.

I claim:

1. An electrophotographic element for use in an electrophotographic copy process comprising a substrate having a photoconductive coating on one surface of the substrate comprising 2,4,7-trinitro-9-fluorenone, a polyvinylcarbazole, and an aromatic anhydride in which the materials are present in the composition of 10 which the coating is formed in the ratio of about 0.49 to 1.23 moles of the 2,4,7-trinitro-9-fluorenone per monomeric unit of the polyvinylcarbazole, and 0.05 to 5.0 parts by weight of the aromatic anhydride per 100 parts by weight of the polyvinylcarbazole.
- 15 2. An electrophotographic element as claimed in claim 1 in which the aromatic anhydride is present in an amount within the range of 0.90 to 1.7 parts by weight per 100 parts by weight of the polyvinylcarbazole.
- 20 3. An electrophotographic element as claimed in claim 1 in which the polyvinylcarbazole is poly-N-vinylcarbazole.
4. An electrophotographic element as claimed in claim 1 in which the aromatic anhydride is phthalic anhydride.
5. An electrophotographic element as claimed in claim 1 in which the aromatic anhydride is 1,2,4,5-benzene-tetracarboxylic anhydride (BT).
6. An electrophotographic element as claimed in claim 1 in which the aromatic anhydride is mellitic trianhydride (MT).
7. An organic photoconductive composition for use in the preparation of a photoconductive coating from which copies can be produced by an electrophotographic process, in which the composition consists essentially of an organic solvent solution of 2,4,7-trinitrofluorenone, a polyvinylcarbazole and an aromatic anhydride in which the materials are present in the solvent solution in the ratio of about 0.49 to 1.23 moles of the trinitrofluorenone per monomeric unit of the polyvinylcarbazole, and 0.05 to 5.0 parts by weight of the aromatic anhydride per 100 parts by weight of the polyvinylcarbazole.
- 35 8. An organic photoconductive composition as claimed in claim 7 in which the aromatic anhydride is present in an amount within the range of 0.90 to 1.7 parts by weight per 100 parts by weight of the polyvinylcarbazole.
- 40 9. An organic photoconductive composition as claimed in claim 7 in which the polyvinylcarbazole is poly-N-vinylcarbazole.
10. An organic photoconductive composition as claimed in claim 7 in which the aromatic anhydride is phthalic anhydride.
- 55 11. An organic photoconductive composition as claimed in claim 7 in which the aromatic anhydride is 1,2,4,5-benzene-tetracarboxylic anhydride (BT).
12. An organic photoconductive composition as claimed in claim 7 in which the aromatic anhydride is mellitic trianhydride (MT).

\* \* \* \* \*